

1

2,711,377

CONSTRUCTION MATERIAL AND METHOD OF  
MAKINGWallace C. Riddell, Berkeley, Calif., assignor to Kaiser  
Gypsum Company, Inc., a corporation of WashingtonNo Drawing. Application September 15, 1952,  
Serial No. 309,747

6 Claims. (Cl. 117—152)

The present invention relates to an improved plasterboard surface, particularly such surface to which it is intended to apply a coating of plaster; and to a process for producing the same.

In building or construction operations, where wallboard, or lath, is installed to form a wall or ceiling, a finish coat of gypsum plaster is applied to the exposed surfaces of the board. These exposed surfaces are fibrous liners, made, for example, of paper, as is well known to the art of manufacturing wallboard or lath wherein a core of cementitious composition, such as set gypsum crystals is formed between fibrous liners. It has been a problem in such work that the fibrous or paper liner has been treated with rosin size which reduces the "suction," or water-absorption, of the liner. This lack of suction seriously hindered bonding of the plaster coating to the liner surface or to the wallboard, as it is generally understood that gypsum plaster adheres to the plasterboard because of the interlocking of the gypsum crystals, as they set, within the fibers of the liner into which a portion of the wet slurry of calcium sulfate hemihydrate has penetrated.

It has been proposed to overcome this disadvantage and to increase the suction by applying to the fibrous or paper surfaces various treating agents, for example, wetting agents, which are intended to enable better penetration of the slurry, or alkalies which saponify and remove some of the sizing and thereby increase water absorption. However, where water absorption is suitably increased, it has been observed that the application of wet plaster to the surfaces of the board often resulted in deformation or sagging of the board, especially in ceiling installations, because an excessive amount of water penetrates into the board, reducing its strength.

It is an object of the invention to improve the adhesion of a plaster coating to the fibrous surface of a wallboard, lath or the like. It is a further object to provide a plaster-receiving fibrous surface of improved water-absorption characteristics; and it is a still further object to provide a plaster-receiving fibrous surface which promotes rapid setting of the plaster and prevention of deformation of the plaster-receiving base.

According to the present invention, it has been found that the above disadvantages are overcome and the aforesaid and other objects are attained by treating the plaster-receiving surface with a solution of calcium hydroxide and a solution of an alkali sulfate, preferably potassium sulfate. The calcium hydroxide is added in an amount to provide from 0.1 to 0.3 lb.  $\text{Ca}(\text{OH})_2$  per 1000 square feet of fibrous or paper surface treated; and the alkali sulfate is added in an amount to provide from 0.3 to 0.6 lb. thereof per 1000 square feet of fibrous or paper surface treated. Preferably, 0.2 lb. calcium hydroxide and 0.45 lb. potassium sulfate are added per 1000 square feet of such surface. The invention will be further described below with special reference to potassium sulfate.

The calcium hydroxide solution can be prepared by dis-

2

solving hydrated, slaked, or unslaked lime in water. The potassium sulfate solution is suitably prepared by dissolving the salt in water. The two solutions can be applied to the surface to be treated independently, but they can conveniently be mixed, or prepared as one treatment mix, and uniformly applied to the surface. The solutions or mixed solutions can be applied to the surface after the board or lath or other fibrous-coated product has been manufactured, or after it has been installed in a wall or ceiling. Alternatively, the solution or solutions can be applied to the exterior liner surface during the manufacture of the product, for example, in the course of manufacture of gypsum wallboard in the manner well known to the art. The solution can be applied by brushing, spraying, rolling, or in any desired manner, and is preferably allowed to dry prior to applying the plaster coating. Preferably, a saturated water solution of calcium hydroxide is employed and a slight excess of  $\text{Ca}(\text{OH})_2$  can be added to insure saturation; and it is preferred to use a 4 to 5% water solution of potassium sulfate.

It is believed, without intending that the present invention be limited by this theory, that the calcium hydroxide and potassium sulfate react metathetically to form, in the presence of water, gypsum ( $\text{CaSO}_4 \cdot 2\text{H}_2\text{O}$ ) and potassium hydroxide. The gypsum (selenite) deposits in the form of minute crystals, uniformly dispersed in the fibers of the liner and upon the liner surface, upon drying, and thereby provides large surfaces of seed crystals which accelerate the setting of the plaster when it is applied, and improve bonding, because of improved penetration and also by accelerated setting time. The potassium hydroxide formed is believed to saponify the sizing of the paper, thereby solubilizing and removing a portion of the size, enabling improved penetration of the plaster slurry into the paper surface and, consequently, stronger bonding thereto. In addition, it is believed that some of the potassium sulfate combines with some of the calcium sulfate to form syngenite crystals which are also deposited in the fibers of the liner. This mineral ( $\text{CaK}_2(\text{SO}_4)_2 \cdot \text{H}_2\text{O}$ ) also has an excellent accelerating effect upon the setting time of calcined gypsum slurry and acts to accelerate the set of later applied plaster. It has been found that the addition of a small amount of potassium sulfate to a calcined gypsum slurry, or of a small amount of selenite (gypsum) crystals to another like slurry, results in acceleration of set in each case from about 35 minutes to about 7 minutes. However, the addition of the same amount of potassium sulfate and of the same amount of selenite crystals to a single batch of slurry effects setting thereof in about 4 minutes. Whatever is the mechanism of the action, however, greatly improved results are obtained by the process and product of the present invention.

The process of this invention is effective in reducing the size in a paper liner for plasterboard, as is demonstrated by examination according to the Cobb paper sizing test (Tech. Assoc. Pulp Paper Industry). In this test, a piece of test paper, 5 inches square, is weighed and then placed in the Cobb Tester and water is added to cover the paper to a depth of one inch at 70° F. After 5 minutes' immersion, the paper is removed and weighed. The amount of water absorbed by the paper is determined by deducting the dry weight from the wet weight. Untreated plasterboard paper tested in this manner absorbed an average of 0.3 gram of water. Another sample of the same paper, but which had been previously treated by application thereto a solution of hydrated lime and potassium sulfate, in an amount to provide 0.2 lb.  $\text{Ca}(\text{OH})_2$  per 1000 square feet surface and 0.45 lb.  $\text{K}_2\text{SO}_4$  per 1000 square feet surface, was tested in exactly the same manner and absorbed 1.44 grams of water, or 4.8 times the amount absorbed by

the untreated paper. The Cobb Tester is made by B. F. Perkins and Sons, Inc., of Holyoke, Mass. and it comprises an iron plate base, a rubber gasket superimposed thereon and a brass ring one inch in depth and of 5-inch inside diameter. The weighed paper to be tested is placed between the gasket and the base of the ring and the ring is then clamped down to effect a seal, and is filled with water at 70° F. providing a one-inch head of water over the paper.

The effectiveness of the process of this invention is also demonstrated by a test which measures the time required for a plasterboard paper liner to absorb 0.1 cc. water at 70° F. In this test, plasterboard paper which had not been treated by the method of this invention absorbed 0.1 cc. water, as delivered from a calibrated burette, in 45 minutes. Another sample of the same paper is surface-treated by brushing it with a water solution providing 0.1 lb. hydrated lime ( $Ca(OH)_2$ ) and 0.3 lb. potassium sulfate, each per 1000 square feet surface, and allowed to dry. The treated paper absorbed 0.1 cc. water in 11 minutes. Therefore, the absorption rate is approximately 4 times as rapid.

It has also been observed that small gypsum crystals accelerate the set of calcined gypsum with water. For example, when one to two pounds of gypsum or selenite crystals in admixed with one ton of calcined gypsum and the whole is then gauged with water, the mass sets in 7 minutes; whereas without the addition of seed crystals, 35 minutes is required for setting time. If the gypsum or selenite crystals are added to the plaster mix itself, the set is not easily controlled and the plaster often sets up before it can be properly applied. According to the present invention it has been found that by this process and in this product, acceleration of the setting time of the plaster is effected after the plaster coating has been applied, and this is apparently brought about by deposition of the seed crystals within and upon the fibrous liner.

In a plant run, gypsum core, paper-lined wallboard is made by preparing a water slurry of calcined gypsum which can also contain minor amounts of modifiers known in this art such as asbestos fibers, foaming agents, water-repellent agents or other modifiers, and the plastic slurry is deposited between fibrous liners or covers, such as paper liners, in a board-forming machine, in the known way. A saturated solution of calcium hydroxide is prepared by thoroughly admixing 9.25 lbs. hydrated lime and 60 gals. of water. In this saturated solution is then dissolved 21.75 lbs. of potassium sulfate. This solution is continuously applied to the surface of the paper to be used for plaster base, as the plasterboard moves down the production line, preferably prior to entering the drier. The solution is applied by means of a felt roll or brush, and at a rate to provide about 0.2 lb. calcium hydroxide and about 0.45 lb. potassium sulfate, per 1000 square feet of board surface. The plasterboard so manufactured was tested in a wall and plaster was applied thereto, which was found to harden in approximately 2 hours, whereas without treatment the same plaster required approximately 4 hours.

Alternatively, a calcium hydroxide solution and a potassium sulfate solution can each be applied to the board, separately and in any desired order. If desired, the solution can be applied to the paper surface after the board has passed through the drier, or at any time prior to application of the plaster. The invention has been described above with reference to potassium sulfate, which is the preferred embodiment because the addition of this salt results in the greatest acceleration of plaster setting, due in part at least, it is believed, to the providing of previously formed seed crystals of syngenite, as well as of gypsum. However, other alkali sulfates, including ammonium sulfate and the sulfates of other alkali metals, are also useful in this invention, either used alone or in admixtures or in admixture with

potassium sulfate. That is, there can be added at least one sulfate chosen from the group consisting of alkali metal sulfates and ammonium sulfate, in the manner which has been described above with more particular reference to potassium sulfate. Of the alkali sulfates, ammonium sulfate is most effective, with the exception of potassium sulfate, the preferred species. The alkali sulfates provide seed crystals of selenite by reaction with the calcium hydroxide. The rosin size is reduced and

10 the seed crystals of gypsum (selenite) or of selenite and syngenite are deposited largely in the outer portion of the fiber liner. The fiber liner can be applied to any plasterboard or gypsum product including particularly gypsum lath and gypsum wallboard. This invention is 15 useful in hastening or accelerating the setting time of gypsum plaster when applied to any fibrous plaster-receiving surface; and exhibits particular advantages in accelerating such setting time and preventing sagging or deformation when applied to fiber or paper coated 20 gypsum lath. The description herein refers to applying solutions but it is to be understood that the solutions can contain some suspended solid material, which can be excess calcium hydroxide to insure saturation of the  $Ca(OH)_2$  solution or it can comprise in the mixed solutions some precipitated gypsum.

In the specification and claims all percentages are by weight unless otherwise indicated. It is to be understood that the above examples have been given for purposes of illustration only and variations and modifications can 30 be made therein without departing from the spirit and scope of the appended claims. By the term "solubilized" used herein is meant to render water-soluble or to convert to water-soluble form, as by saponification.

Having now described the invention, what is claimed 35 is:

1. Process for improving the plaster-bonding properties of a fibrous plaster-receiving surface which comprises applying directly to said surface, substances in aqueous solution consisting essentially of calcium hydroxide in 40 an amount to provide from 0.1 to 0.3 lb. of calcium hydroxide per 1000 sq. ft. of said surface and at least one sulfate selected from the group consisting of alkali metal sulfates and ammonium sulfate in an amount to provide from 0.3 to 0.6 lb. total of said sulfate per 1000 sq. ft. 45 of said surface.

2. A process as in claim 1 wherein there are applied to the fibrous surface 0.2 lb. of calcium hydroxide and 0.45 lb. of potassium sulfate per 1000 sq. ft. of surface.

3. Process for improving the plaster-bonding properties of the paper surface of a paper coated gypsum product which comprises preparing a saturated water solution consisting essentially of calcium hydroxide, dissolving potassium sulfate in said solution, and applying the said solution directly to the surface of said paper coated 50 gypsum product in amount to provide from 0.1 to 0.3 lb. of calcium hydroxide and from 0.3 to 0.6 lb. of potassium sulfate per 1000 sq. ft. of paper surface.

4. Process for improving the plaster-bonding properties of the paper surface of a paper coated gypsum product which comprises applying directly to the paper surface a water solution consisting essentially of calcium hydroxide in an amount to provide from 0.10 to 0.30 lb. of calcium hydroxide per 1000 sq. ft. of surface, and a water solution consisting essentially of potassium sulfate in an 60 amount to provide from 0.3 to 0.6 lb. of potassium sulfate per 1000 sq. ft. of surface.

5. Plaster board having an improved plaster-receiving paper surface comprising a rosin-sized paper liner containing a small amount of uniformly dispersed finely divided gypsum therein, the gypsum having been deposited and the said rosin-size having been partially saponified by a process according to claim 1.

6. Plaster board having an improved plaster-receiving paper surface comprising a rosin-sized paper liner containing a small amount of uniformly dispersed finely di-

vided syngenite therein, the syngenite having been deposited and the said rosin-size having been partially saponified by a process according to claim 1.

## References Cited in the file of this patent

5 848,916  
1,451,485  
1,738,976  
1,868,372  
2,034,435  
2,526,537

## UNITED STATES PATENTS

107,687 Hudson Sept. 27, 1870

|          |       |               |
|----------|-------|---------------|
| Monin    | ----- | Apr. 2, 1907  |
| Wootton  | ----- | Apr. 10, 1923 |
| Vivas    | ----- | Dec. 10, 1929 |
| Swift    | ----- | July 19, 1932 |
| Heritage | ----- | Mar. 17, 1936 |
| Camp     | ----- | Oct. 17, 1950 |